

Patented Dec. 7, 1926.

1,609,882

# UNITED STATES PATENT OFFICE.

JOHN NEVIN POMEROY, OF PHILADELPHIA, PENNSYLVANIA.

## PROCESS OF TREATING ZINC WASTE.

No Drawing.

Application filed May 6, 1922. Serial No. 559,056.

My invention relates to a process of treating zinc waste, for recovering zinc materials, which are suitable for use in the manufacture of lithopone, while the same may be used for other purposes.

An important object of the invention is to provide a process of the above mentioned character, for obtaining zinc materials, having a low content of chlorides.

In the manufacture of lithopone, zinc materials, such as zinc ash, zinc skimmings from galvanizing processes, zinc residues from vat wastes, and zinc residues from other industries, are employed. These zinc materials ordinarily contain a considerable amount of chlorides. The chloride content in such materials has been found to be injurious to the lithopone produced, inasmuch as the presence of the same causes the lithopone to dis- 20 color, when exposed to light.

The zinc materials hereinbefore referred to, ordinarily contain .1 (one-tenth) per cent to 6 or 7 (six or seven) per cent of chloride. I have discovered that zinc materials containing more than .1 (one-tenth) per cent of chloride impart injurious properties to the lithopone, as above stated.

Certain zinc waste, such as zinc ash, zinc skimmings from the galvanizing process, zinc residue from vat wastes, and zinc residues from other industries, contain from 35 (thirty-five) to 85 (eighty-five) per cent of zinc, as metallic zinc, zinc oxid, zinc chloride, zinc sulphate, etc., or a mixture of them all. The remaining portion of the zinc waste comprises impurities, such as chlorides, sal-ammoniac, iron, sulphites or organic material.

My process comprises first working this zinc waste or zinc materials up to a proper physical condition, for subsequent treatment.

The material ordinarily occurs in large lumps or the like, and it is first passed through an ore crusher, which serves to break up the large lumps. These large lumps contain large pieces of metallic zinc, which are freed by the breaking action. The broken material is then passed through a coarse screen, of an inch or an inch and a half mesh, and the large lumps of metallic zinc are caught upon the screen and thus separated from the material. The material thus passing through the screen is now subjected to a second breaking action or grinding, and for this purpose I preferably pass the same through a ball mill, or any other

suitable mill, to crush the same. The material is preferably crushed to a fineness so that it will pass through a 40 (forty) mesh screen. The zinc metallics are caught upon the top of this screen and thus separated out from the material passing through the screen. The fine material thus screened is passed over a magnetic separator, which eliminates any small particles of iron, that may have passed through the screens. The material may be mechanically worked up in different ways, and the invention is not restricted to the precise method stated. The material may be handled in a wet way, and the zinc metallics removed by levigation.

The zinc material, thus mechanically treated, is now subjected to the action of sulphuric acid. The material is therefore introduced into a suitable mixer, and is there treated with strong sulphuric acid. The proportions of the sulphuric acid and the zinc material will vary depending upon the nature of the zinc material, and it is often necessary, to obtain satisfactory results, to properly vary the amount of acid and zinc materials, as may be determined by experience. After considerable experimentation, to secure the maximum elimination of chlorides for a high grade zinc ash containing 80 (eighty) per cent zinc and 5 (five) per cent chlorides, I treat 800 pounds of zinc material with 600 pounds of strong sulphuric acid. The invention is of course in no sense restricted to these precise proportions, as they may be varied, as indicated.

The chemical reaction which takes place during this treatment with sulphuric acid serves to eliminate substantially 90 (ninety) per cent of the chlorides present in the zinc material.

A mixture of  $Zn$ ,  $ZnO$ ,  $ZnCl$ , and  $NH_4Cl$  is employed plus sufficient  $H_2SO_4$  to combine with the chlorides present, but not sufficient to completely combine with all of the  $Zn$  present. As a result of this mixture,  $Zn$ ,  $ZnO$  and  $ZnSO_4$  plus  $HCl$ ,  $(NH_4)_2SO_4$  plus  $H_2O$  is obtained. The  $H_2O$  and the  $HCl$  are volatilized.

The heat of the reaction causes a considerable rise in temperature, from about 60° F. to 180° F. Ninety per cent of the volatiles contained within the material, such as hydrochloric acid and ammonium chloride are thus volatilized and driven off from the material. I have found that it is not nec-

essary to add sufficient sulphuric acid to completely combine with all of the zinc present, but the addition of an amount of acid not sufficient to combine with all of the zinc present, will eliminate at least ninety per cent of the chlorides at this step in the process, and thus reduce the chloride content of the zinc material from 6 (six) per cent to approximately .5 (five-tenths) per cent.

10 The material thus treated and containing .5 (five-tenths) per cent of chloride, still possesses too high a chloride content, to be successfully used in making a high class lithopone. I have found that in order to reduce the remaining chloride content in the material, so that the same will be within the limits of .05 (five-hundredths) to .1 (one-tenth) per cent. that it is necessary to subject the treated material to a roasting 20 operation.

The material in the mixer, after it has had sufficient time to react with the sulphuric acid, is in the form of a powder. This powder is dropped from the mixer into 25 a suitable hopper, from which it is fed to the roaster. While any suitable form of roaster may be used, I prefer to employ a rotary furnace, while an ordinary hand grate furnace is also suitable. On account of economy in 30 labor and fuel, the rotary type of furnace is desirable. The material is now passed into the rotary furnace wherein it is subjected to a temperature varying from 500 (five hundred) degrees F. to 2000 (two thousand) 35 degrees F., depending somewhat upon the nature of the material being treated. As a matter of fact, after considerable experimentation, I have found that the temperature may be widely varied. The best 40 method for heating the roaster or rotary furnace, I have found, to be by a counter heat, the heat traveling longitudinally of the furnace in an opposite direction to the longitudinal travel of the material. It is preferred to use either oil or gas, for fuel, atomizing with air, so that at all times, an oxidizing atmosphere may be obtained, which 45 has been found advantageous to the successful practice of the process.

50 The effect of heat upon the treated material is to partly break down some of the sulphates present, which in turn attack the small amount of the chlorides remaining, and these chlorides, due to the temperatures, are 55 volatilized and driven off from the material. I have found an oxidizing atmosphere desirable, because owing to the presence of organic material and of particles of metallic zinc, there is a tendency to reduce the sulphates to free sulphur or sulphides, which results in a considerable loss of sulphur, and a product that is not very satisfactory for lithopone manufacture. The finished material as it leaves the roaster or rotary furnace, will vary somewhat in chemical compo- 60 65

sition, depending upon the amount of acid used, the original zinc content of the material, and certain impurities which cannot be eliminated by the process. The sulphate content of the finished material will, in some instances, vary between the limits of 10 (ten) to 45 (forty-five) per cent depending upon the character of the zinc waste treated, and is a valuable addition to the treated material, because it can be used with zinc in lithopone manufacture. The chloride content will be reduced from say a maximum content of 6 (six) per cent in the original material to from .05 (five hundredths) per cent to .1 (one-tenth). This material is satisfactory for zinc crude, used in the manufacture of a high grade lithopone.

The zinc material may occur in such form, so as to be free from lumps or metallic zinc particles, so that the mechanical separation may be dispensed with.

It is to be understood that the form of my invention herewith shown and described is to be taken as a preferred example of the same, and that various changes may be resorted to in the order of the steps of the process, and that chemical equivalents may be employed without departing from the spirit of the invention or the scope of the subjoined claims.

Having thus described my invention, I claim:

1. The process of treating zinc waste containing a high chloride content to lower such content, which comprises mechanically separating out the metallic zinc, subjecting the material thus treated to the action of sulphuric acid to remove the greater portion of the chloride content, and then roasting the material to volatilize out further of the remaining chloride content.

2. The method of treating zinc waste for obtaining a material for use in the production of lithopone, said material containing a major portion of zinc material having a low chloride content, which comprises subjecting the zinc waste to the action of heat at approximately 2000° F. in the presence of an oxidizing atmosphere whereby the major portion of the chloride content is volatilized out, and recovering the zinc material having a low chloride content.

3. The process of treating zinc waste containing a high chloride content to lower the same, which consists in breaking the material up into relatively large lumps, screening the material for separating out the metallic zinc lumps, subjecting the material to a grinding operation to finely divide the same, screening the finely divided material to separate out metallic zinc particles, separating out the iron particles in the material, subjecting the material to the action of sulphuric acid to remove the greater portion of the chloride content, and roasting

the material thus treated to volatilize out further of the remaining chloride content.

4. The method of treating zinc waste for obtaining a material for use in the production of lithopone, which comprises subjecting the zinc waste to the action of heat between substantially 500° F. and 2000° F. in the presence of an oxidizing atmosphere whereby the major portion of the chloride content is volatilized out and a zinc material relatively high in zinc and low in chloride content is produced, and recovering said zinc material.

5. The process of treating zinc waste for obtaining zinc material having a low chloride content, which comprises subjecting the zinc waste to the action of heat between substantially 500° F. and 2000° F. in the presence of an oxidizing atmosphere to produce a zinc material relatively high in zinc and low in chloride material thus separating the chloride material from the zinc material, and recovering said zinc material.

6. The method of treating zinc waste for obtaining a material for use in the production of a sun proof lithopone, such material containing a major portion of zinc material having a low chloride content, which comprises subjecting the zinc waste to the action of heat upward to 2000° F. in the presence of an oxidizing atmosphere to produce a zinc material relatively high in zinc and low in chloride material and thus separating the chloride material from the zinc material, and recovering said zinc material.

7. The method of treating zinc vat waste for obtaining a material for use in the production of a sun proof lithopone, such material containing a major portion of zinc material having a low chloride content, which comprises subjecting the zinc waste to the action of heat between substantially 500° F. to 2000° F. in the presence of an oxidizing atmosphere to produce a zinc material relatively high in zinc and having

a chloride content between .05 and .1 per cent and thus separating the chloride content from the zinc material, and recovering said zinc material.

8. The method of treating zinc vat waste for obtaining a material for use in the production of a sun proof lithopone, such material containing a major portion of zinc material having a low chloride content, which comprises separating out the major portion of the chloride content and obtaining a material still possessing too high a chloride content, and then subjecting such material to the action of heat between approximately 500° F. to 2000° F. in the presence of an oxidizing atmosphere to produce a zinc material relatively high in zinc and having a chloride content between .05 and .1 per cent and thus separating the chloride content from the zinc material, and recovering said zinc material.

9. The method of treating zinc vat waste for obtaining a material for use in the production of a sun proof lithopone, such material containing a major portion of zinc material having a low chloride content, which comprises mechanically separating out the metallic zinc from the zinc waste, subjecting the material thus treated to the action of sulphuric acid to separate out the major portion of the remaining chloride content and obtaining a material still possessing too high a chloride content, and then subjecting such material to the action of heat between approximately 500° F. to 2000° F. in the presence of an oxidizing atmosphere to produce a zinc material relatively high in zinc and having a chloride content between .05 and .1 per cent and thus separating out the chloride content from the zinc material, and recovering said zinc material.

In testimony whereof I affix my signature.

JOHN NEVIN POMEROY.